

## UNITED STATES PATENT OFFICE

2,045,788

FUEL FOR HIGH PRESSURE LIQUID  
FUEL INJECTION ENGINES

George M. Maverick, Elizabeth, N. J., assignor to  
Standard Oil Development Company, a corpora-  
tion of Delaware

No Drawing. Application July 11, 1933,  
Serial No. 679,891

## 1 Claim. (Cl. 44—9)

This invention relates to improved fuels for engines employing high pressure liquid fuel injection, such as the Diesel and spark ignited types, and more particularly it relates to such fuels containing extreme-pressure lubricating ingredients and also to methods of producing such fuels.

There have been many attempts to develop high-speed Diesel engines for various particular uses such as automotive, aviation, railroad or stationary use, but these have not been attended with the desired degree of success. This partial failure is, to a certain extent, due to the inability to use sufficiently low viscosity fuels as they are deficient in lubricating value with the result that fuel pumps and injection valves fail after a short period of operation. It is an object of the present invention to overcome these difficulties.

Internal combustion engines are of two general types: those employing the Otto cycle as in the ordinary automobiles and those of the auto-ignition type which use the Diesel cycle. The principal difference between these two types is that in the Otto cycle, air and fuel are mixed in a carburetor and the mixture is admitted to the cylinder, compressed by the piston to between 50 and 225 pounds per square inch and then ignited by an electric spark; whereas in the Diesel cycle, air alone is first admitted to the cylinder and compressed to a much higher pressure, i. e., between 500 and 2,000 pounds per square inch, and then liquid fuel is injected and the mixture automatically ignites due to the increased temperature which resulted from the high compression of the air.

It is therefore apparent that in using the Diesel cycle the liquid fuel must be injected under pressures sufficiently high to overcome the pressure of the compressed air already in the cylinder. Under these conditions, it is difficult to lubricate the fuel injection pumps, valves and nozzles. However, for ordinary Diesel operation, it is desirable to use a fuel of as low a viscosity as possible. There are many reasons for this selection, the most important being that better injection is obtained, and that the auto-ignition temperature is lower. Unfortunately, petroleum fuels of such low viscosities have substantially little lubricating value, and since the fuel in most engines of this type is also the lubricant for the injection pumps and valves, it has been found necessary to employ oils of viscosities sufficiently high to give the desired lubrication. However, due to such high viscosity, injection of this fuel through the nozzle to produce the most efficient spray is difficult, and engines of this type suffer through im-

proper atomization and combustion, too high auto-ignition temperature (A. I. T.), difficult starting, waste of fuel, etc.

This invention involves the elimination of such difficulties in not only the true Diesel type of auto-ignition engines, but also in the other modified prime movers such as the Hesselman and Atlas engines which employ the Otto cycle involving liquid fuel injection and spark ignition.

Broadly, the invention consists in adding to the fuel certain materials which will increase its lubricity though without appreciably increasing its viscosity or having any other harmful effects. These materials are generally termed extreme pressure lubricants or load carrying agents and their important characteristic consists in the fact that only small amounts need be added to the fuel to increase its oiliness to the desired extent. In this respect they differ from the mineral oils which owe their lubricating powers mainly to their viscosity. Generally, from  $\frac{1}{2}\%$  to 2% is sufficient, although the actual amount added depends upon the materials blended. Suitable materials to be added include reactive sulfur compounds, alone or with tin and lead compounds.

Certain organic acids and esters may also be used. The acids should be of the naphthenic acid type, and usually should comprise molecules containing 8 to 10 carbon atoms or preferably more. The esters should have a relatively high boiling point, that is, in the range of or above the temperature of the combustion chamber. Such high-boiling esters may be of the cyclic, heterocyclic, aliphatic or mixed types. Esters having a boiling point above 150° C., claimed in co-pending application Ser. No. 600,828 by Per K. Frolich, include inter alia amyl butyrate (B. Pt. 176° C.), butyl naphthenate, phenyl acetate (B. Pt. 196° C.), etc. Still higher boiling esters are claimed in co-pending application Ser. No. 667,039, filed April 20, 1933, by Jones I. Wasson, as a gum flux or upper cylinder lubricant in a motor fuel; some of the specific esters disclosed are amyl and heptyl stearate, amyl cinnamate (B. Pt. 572° F.) and secondary amyl ester of mono-toluene stearic acid (B. Pt. between 700—800° F.). Such compounds must have sufficiently high boiling points so as not to boil off at the temperature of the cylinder head. Furthermore, they must be sufficiently stable so as not to decompose to insoluble products, thereby causing clogging of the injection nozzle.

Substances comprising sulfur should be sufficiently unstable to be of the active or corrosive type, since otherwise, little if any increase in

- lubricity is obtained. In preparing sulfur compounds, sulfur may be cooked with paraffin wax or a sulfurized mineral oil or vegetable oil may be produced, in which the sulfur is present in a chemically combined and reactive condition. Generally, the disulfides are not satisfactory, whereas the tetrasulfides are. In using corrosive compounds, especially those containing sulfur, care must be taken that tanks and feed lines, etc. are made of suitable material as the active sulfur compounds corrode metals such as zinc and copper. Lead soaps, such as lead oleate, may be used as suitable lead compounds.
- Mixtures or combinations of the above types of extreme pressure lubricating ingredients may be used, for example, a mixture such as sulfurized oil and lead oleate; and also mixtures of any such ingredients with some of the organic acid and ester type mentioned above may be used.
- In this way a superior lubricating property is imparted to the fuel with which those ingredients are mixed. Specific examples of various illustrative combinations will be given herein-after.
- The fuel to be used may be a single type petroleum hydrocarbon fuel such as gas oil, kerosene or gasoline, or may be a blended fuel comprising petroleum hydrocarbons as well as other types of fuel such as benzol, alcohol, etc. A special gasoline type fuel, known as safety fuel, is particularly useful in the present invention. This safety fuel which is claimed separately in co-pending application Ser. No. 464,450 by F. A. Howard has a boiling range between the approximate limits of 300 to 550° F. Its chief advantage lies in the absence of the very low boiling ends which are apt to create a fire hazard. Such a specially cut naphtha, free from both light and heavy ends, may consist either of the hydrocarbons normally present in ordinary gasoline or a cracked gasoline or may preferably be produced by hydrogenation of various types of hydrocarbons as is more fully described in the Howard application referred to.
- Likewise, instead of using the usual Diesel fuels which generally have gravities of 26 to 30° A. P. I. and viscosities in the neighborhood of 50 seconds Saybolt, it is possible to employ fuels of 40 to 45° A. P. I. gravity and 300 to 450 refined oil viscosity (30 to 35 Saybolt).

In preparing the improved fuels according to the invention, the addition agent is added to the fuel base in amounts varying generally from 0.1% up to 5.0% or so, depending upon the type of fuel and addition agents as well as the design of the high pressure injection engine in which the fuel will be burned. Generally, with the heavier types of fuel, only a small amount of load carrying agent is necessary, whereas with the lighter hy-

drocarbon fuels of the gasoline type a larger amount of addition agent will be required. These addition agents may either be added directly to the large bulk of fuel base or they may be incorporated into a small amount of the fuel base and then this mixture stirred into the larger bulk of the fuel base.

For the sake of illustration only and without intention to be limited thereby, the following examples are given:

*Example 1*

|                                | Percent |
|--------------------------------|---------|
| Gas oil (40° A. P. I. gravity) | 99.0    |
| Butyl acetyl ricinoleate       | 0.1     |
| Sulfurized pine or lard oil    | 0.9 15  |
|                                | 100.0   |

*Example 2*

|                                     | Percent |
|-------------------------------------|---------|
| Safety fuel (300 to 550° F. B. Pt.) | 99.0 20 |
| Sulfur compound                     | 0.5     |
| Lead soap                           | 0.5     |
|                                     | 100.0   |

There may also be added to these auto-ignition engine fuels any other substances desired, for example, materials adapted to facilitate the ignition of the fuel, such as nitro compounds, knock inducers, dyes, inhibitors, or gum fluxes such as the high-boiling mineral oil of naphthenic type as disclosed in the co-pending application of Sloane and Wasson, Ser. No. 658,153 filed February 23, 1933.

In the appended claims the expressions "a fuel for high pressure liquid fuel injection engines" and "a Diesel fuel" are intended to mean fuels having a sufficient lubricity or load carrying capacity that they are adapted to prevent excessive wear of fuel injection pumps and other moving parts in contact with the fuel under the high pressures used in such engines.

It is not intended that the invention be limited to the specific examples given nor to any theory of the operation of the invention but it is desired to claim broadly all inherent novelty in the invention.

I claim:

A fuel for Diesel and other high pressure liquid fuel injection engines which comprises a major proportion of a light hydrocarbon liquid having a viscosity substantially as great as that of gas oil and containing 0.5 to 5.0% of a compound containing a substantial amount of chemically combined sulfur in a reactive condition, said fuel also containing about 0.5 to 2.0% of a compound of a metal of the group consisting of tin and lead, which compound is capable of reacting with the sulfur compound to give increased lubricity.

GEORGE M. MAVERICK.